

**1**

3,355,363

**METHOD OF PRODUCING A NONAGGLOMERATING CHAR FROM A STRONGLY CAKING COAL**

Stanley J. Gasior, Pittsburgh, and Albert J. Forney, Coraopolis, Pa., assignors to the United States of America as represented by the Secretary of the Interior  
No Drawing. Filed Feb. 14, 1964, Ser. No. 345,053  
9 Claims. (Cl. 201—9)

**ABSTRACT OF THE DISCLOSURE**

A nonagglomerating char is produced from a particulate caking coal by contacting the coal in a fixed bed at its initial softening temperature with a gas containing small quantities of oxygen for a period of one to three hours.

The invention herein described and claimed may be manufactured and used by or for the Government of the United States of America for governmental purposes without the payment of royalties thereon or therefor.

This invention relates to treatment of caking coals to form a nonagglomerating char.

As natural gas reserves in the United States continue to dwindle, the most likely substitute is a synthetic high-B.t.u. gas produced from coal. Presently, fixed-bed pressure gasification appears to be most attractive for producing a high-B.t.u. gas. A gas with high methane content may thus be made with low oxygen requirements. Previously, however, strongly caking coals could not be gasified in this manner since they agglomerate when heated through a temperature range at which they become plastic, rendering the gasifier inoperable. Coals from the vast deposits in the East and Midwest, where the largest markets for a high-B.t.u. gas exist, are highly caking.

Existing commercial producers of noncaking coal-chars require mechanical devices such as a rotating kiln, chain grates, jiggling grates, rotating screws, etc., to prevent the strongly caking coals from fusing into one solid mass while being taken through the plastic temperature range. These devices necessitate high capital investment.

Fluidized bed processes, such as that disclosed in U.S. Patent No. 2,805,189, in which the fluidized bed is treated with an oxygen-containing gas have also been employed to prevent agglomeration of coal in processes such as carbonization, gasification, hydrogenation, etc. These fluidized bed processes have the disadvantage that the coal size is critical, and in addition require a costly briquetting step to increase the size of the small particles of char produced in the fluidized treatment. Another disadvantage of the fluidized bed process is that the treating gas velocity is critical, thus placing a strict operational limitation on fluidized treatment.

Previous attempts to produce a noncaking char in a fixed bed, without the use of mechanical devices as described above, have met with little success.

It is therefore an object of the present invention to provide a fixed bed process for producing nonagglomerating char from a strongly caking coal that is simple, noncritical and inexpensive.

**2**

It has now been found that this object may be accomplished by means of a controlled heating of the caking coal in an atmosphere of an inert gas that contains a small amount of oxygen. It has been found that the coal must be treated with the oxygen-containing gas for a period of time at its initial softening and swelling temperature prior to being heated through its plastic temperature.

As indicated by the terms, the initial softening and swelling temperature is that temperature (or range of temperatures) at which the particles of coal begin to soften, swell and thereby fill the voids between the particles of coal. Conventional tests for determining this temperature utilize a flow of gas through the coal, the softening and swelling temperature being indicated by an increase in the differential pressure across the fixed-bed of coals due to filling of the aforementioned voids between the coal particles.

Following this treatment at the softening and swelling temperature, the coal particles may be taken through their plastic temperature range, i.e., the temperature at which the coal becomes plastic and resembles a paste or dough in which the particles flow within each other, in a fixed bed without caking, fusing or agglomerating. The coal particles may then also be exposed to a hydrogen-rich atmosphere at elevated temperatures and pressures in a fixed bed to produce a high-B.t.u. gas without agglomerating.

It has been found that a process in which the coal is rapidly heated to its initial softening and swelling temperature and then held at this temperature for a period of time in an atmosphere of inert gas containing a small amount of oxygen generally gives very satisfactory results. The period of time will depend on the type of coal treated as well as the amount of coal, particle size, treatment gas, etc., and is best determined empirically. It has been found that a period of treatment of about 3 hours is sufficient to prevent agglomeration in the case of the Pittsburgh seam coal employed in the examples below. Different time periods may be optimum for other types of coal, e.g., high volatile "B" bituminous Illinois No. 6 requires only about 80 minutes while for Pocahontas No. 4, a low volatile bituminous coal, a period of about 120 minutes is optimum, as compared to 180, 190 and 200 minutes, respectively, for the high volatile "A" bituminous coals from the Upper Freeport, Taggart and Sewickley seams. Treatment times in the range of 1 to 3 hours have given satisfactory results for the coals tested. The coal may then be rapidly heated through its plastic temperature in the same atmosphere. The softening temperature and plastic temperature will usually encompass a range of temperatures and will vary considerably with the type of coal treated but may be readily determined by those skilled in the art if not previously known. The source, analysis, free swelling index, initial softening and maximum pretreatment temperatures are shown in Table 1.

Alternatively, coal may be effectively pretreated by rapid heating to its softening temperature in the oxygen-containing inert atmosphere followed by prolonged heating, as for example about 3 hours, through its plastic range in the same atmosphere.

TABLE 1.—SOURCE, ANALYSIS, FREE SWELLING INDEX, INITIAL SOFTENING AND MAXIMUM PRETREATMENT TEMPERATURES OF COALS TESTED

| County, bed, mine                                | Proximate, percent |                 |              |      | Ultimate, percent |      |     |      |     | Initial softening temp., °C. | Free swelling index | Maximum pretreatment temp., °C. |
|--------------------------------------------------|--------------------|-----------------|--------------|------|-------------------|------|-----|------|-----|------------------------------|---------------------|---------------------------------|
|                                                  | Moisture           | Volatile matter | Fixed carbon | Ash  | H                 | C    | N   | O    | S   |                              |                     |                                 |
| Illinois                                         |                    |                 |              |      |                   |      |     |      |     |                              |                     |                                 |
| Franklin, Illinois No. 6, Ben No. 21             | 8.0                | 35.4            | 50.0         | 6.6  | 5.5               | 70.6 | 1.7 | 14.7 | 0.9 | 350                          | 4.5                 | 430                             |
| Pennsylvania                                     |                    |                 |              |      |                   |      |     |      |     |                              |                     |                                 |
| Allegheny, Pittsburgh, U.S. BuMines Experimental | 2.5                | 35.6            | 54.3         | 7.6  | 5.3               | 75.8 | 1.5 | 8.2  | 1.6 | 360                          | 8.5                 | 430                             |
| Butler, Upper Freeport, Coal Hollow No. 2        | 1.7                | 35.3            | 55.9         | 7.1  | 5.3               | 76.9 | 1.5 | 7.9  | 1.3 | 350                          | 8.0                 | 430                             |
| Virginia                                         |                    |                 |              |      |                   |      |     |      |     |                              |                     |                                 |
| Wise, Taggart, Dixiana                           | 1.4                | 33.8            | 62.3         | 2.5  | 5.3               | 82.8 | 1.5 | 7.2  | 0.7 | 360                          | 8.5                 | 430                             |
| West Virginia                                    |                    |                 |              |      |                   |      |     |      |     |                              |                     |                                 |
| McDowell, Pocahontas No. 4, Bartley No. 1        | 2.7                | 14.8            | 76.5         | 6.0  | 4.4               | 83.3 | 1.3 | 4.5  | 0.5 | 470                          | 6.5                 | 510                             |
| Monongalia, Sewickley, Christopher No. 5         | 1.1                | 36.7            | 50.9         | 11.3 | 5.1               | 73.3 | 1.5 | 6.2  | 2.6 | 360                          | 8.0                 | 430                             |

It has additionally been found that the pretreatment techniques as developed at atmospheric pressure works equally well at pressures up to 300 p.s.i.g. Optimum pressure will also vary with the type of coal, amount, particle size, treatment gas, etc.

The specific composition of the gas used in the pretreatment is not critical except that it must contain the required small amount of oxygen. The optimum amount of oxygen will also depend on the type of coal, as well as other variables discussed above, and is best determined empirically. Generally, the oxygen content will be in the range of about 0.5 to about 3.0%. For economic purposes a source of cheap inert gas such as flue gas, steam, carbon dioxide, or nitrogen, containing some air or oxygen is preferred.

The invention is more specifically described but is not intended to be limited by the following examples.

#### Examples 1-11

Reactants, reaction conditions and results of these examples are given in Table 2. A Pittsburgh seam strongly

caking coal from a Bruceton, Pennsylvania mine having the analysis given in Table 3, below, and a particle size of about  $\frac{1}{4} \times \frac{1}{2}$  inch was used in Tests Nos. 1, 2, 3, 5, 30 7, 9 and 11. Coal having a particle size range of about  $\frac{1}{8}$  to about  $\frac{1}{2}$  inches is satisfactory for use in the process. The coal used in the other examples is shown in Table 2. The coal was treated in a fixed bed in a  $3\frac{1}{2}$  diameter vessel with a bed height as shown in Table 2. In the 35 examples the treatment gas entered the bottom of the reaction vessel and passed upwardly through the bed of coal at atmospheric pressure. Gas velocity through the coal bed may range from about 0.6 to about 12 feet per second. However, treatment of the coal with gas passing downwardly through the bed has been found to be 40 equally successful.

Analyses of the coal used in the tests and the coal or char produced in the pretreatment are given in Table 3. The inert gas used to quench the coals in Examples 2, 4, 45 6, 8, 10 and 11 was a mixture of 88 percent nitrogen and 12 percent carbon dioxide with a trace of oxygen. Other inert gases such as nitrogen alone could be used for this purpose.

TABLE 2

| Test No. | Coal charge, grams         | Bed height, inches | Type of treat. gas and amt., s.c.f.h. | Treatment Conditions                                                                                                                                                                                | Results                                                                              |
|----------|----------------------------|--------------------|---------------------------------------|-----------------------------------------------------------------------------------------------------------------------------------------------------------------------------------------------------|--------------------------------------------------------------------------------------|
| 1        | 600                        | 6                  | Steam + O <sub>2</sub> , 300+3.       | Coal heated from 30° to 360° C. in $\frac{1}{2}$ hr. with steam plus oxygen then cooled to 100° C with N <sub>2</sub> in $\frac{1}{2}$ hr.                                                          | No fusion. No apparent weight loss. Coal appeared same as charged.                   |
| 2        | 600                        | 6                  | Steam + O <sub>2</sub> , 300+3.       | Coal heated from 30° to 360° C. in $\frac{1}{2}$ hr. to 430° C. in 3 hr. with steam plus oxygen; cooled to 100° C. in $\frac{1}{2}$ hr. with inert gas.                                             | No fusion. 18.5% weight loss. Bed expanded 50%. Char flowered as freely as raw coal. |
| 3        | 600                        | 6                  | Air, 300                              | Coal heated to 200° C. in $\frac{1}{2}$ hr. held at 200° C. for 16 hr., then cooled to 100° C. in $\frac{1}{2}$ hr. with air.                                                                       | No fusion; no apparent weight loss. Coal appeared same as charged.                   |
| 4        | Coal from test No. 3, 440. | 4                  | Steam, 300                            | Coal heated from 30° to 430° C. in 75 min. with steam; cooled to 100° C. in $\frac{1}{2}$ hr. with inert gas.                                                                                       | Char fused into one solid mass of highly porous char.                                |
| 5        | Coal from test No. 3, 440. | 20                 | Air 400                               | Coal heated from 30° to 300° C. in 3 hr. and held at 300° C. for 8 hr.; then cooled to 100° C. in $\frac{1}{2}$ hr. with air.                                                                       | No fusion. 3.5% weight loss. Coal appeared same as charged.                          |
| 6        | Coal from test No. 5, 600. | 6                  | Steam + O <sub>2</sub> , 400+5.       | Coal heated from 30° to 430° C. in 75 min. with steam and O <sub>2</sub> , then cooled to 100° C. in $\frac{1}{2}$ hr. with inert gas.                                                              | Char fused into one solid mass with some discernible particles.                      |
| 7        | 600                        | 6                  | Air, 500                              | Coal heated from 30° to 340°-350° C. in 2 hr. and held at 340-350° C. for 8 hr.; then cooled to 100° C. in $\frac{1}{2}$ hr. with air.                                                              | No fusion. 4.5% weight loss. Coal appeared same as charged.                          |
| 8        | Coal from test No. 7.      | 5                  | Steam + O <sub>2</sub> , 400+5.       | Coal heated from 30° to 430° C. in 80 min. with steam plus O <sub>2</sub> , then cooled to 100° C. in $\frac{1}{2}$ hr. with inert gas.                                                             | Char fused into one solid mass with some discernible particles.                      |
| 9        | 600                        | 6                  | Air, 300                              | Coal heated to 200° C. in $\frac{1}{2}$ hr.; held at 200° C. for 16 hr., then cooled to 100° C. in $\frac{1}{2}$ hr. with air.                                                                      | No fusion; no apparent weight loss. Coal appeared same as charged.                   |
| 10       | Coal from test No. 9, 400. | 4                  | Steam + O <sub>2</sub> , 300+3.       | Coal heated from 30° to 430° C. in 75 min. with steam plus 1% oxygen; then cooled to 100° C. in $\frac{1}{2}$ hr. with inert gas.                                                                   | Char fused into one solid mass of highly porous char.                                |
| 11       | 600                        | 6                  | Steam + O <sub>2</sub> , 300+3.       | Coal heated from 30° to 360° C. in 15 min.; held at 360°-370° C. for 180 min. then heated to 430° in 30 min. with steam plus 1% oxygen. Char cooled to 100° C. in $\frac{1}{2}$ hr. with inert gas. | No fusion; 18.4% weight loss. Char flowered as freely as coal.                       |

TABLE 3

| Components                             | Pittsburgh seam PGH | 1      | 2               | 3      | 5      | 7      | 8      | 9      | 10     | 11              |
|----------------------------------------|---------------------|--------|-----------------|--------|--------|--------|--------|--------|--------|-----------------|
| Moisture.....                          | 1.4                 | 0.5    | 0.6             | 0.3    | 0.4    | 0.5    | 0.3    | 0.5    | 0.7    | 0.7             |
| Volatile matter.....                   | 37.0                | 35.7   | 20.1            | 37.5   | 36.9   | 35.1   | 36.1   | 37.5   | 25.4   | 20.2            |
| Fixed carbon.....                      | 57.0                | 57.0   | 70.9            | 57.0   | 56.7   | 58.7   | 56.3   | 57.0   | 66.3   | 73.2            |
| Ash.....                               | 4.6                 | 6.8    | 8.4             | 5.2    | 6.0    | 5.7    | 7.3    | 5.0    | 7.6    | 5.9             |
| H.....                                 | 5.4                 | 5.1    | 4.1             | 5.1    | 4.8    | 4.6    | 5.0    | 5.1    | 4.6    | 4.1             |
| C.....                                 | 79.6                | 78.7   | 77.9            | 77.8   | 77.0   | 76.8   | 77.7   | 77.8   | 77.8   | 79.7            |
| N.....                                 | 1.6                 | 1.6    | 1.8             | 1.6    | 1.6    | 1.7    | 1.6    | 1.6    | 1.8    | 1.8             |
| O.....                                 | 7.8                 | 6.2    | 6.4             | 9.3    | 9.4    | 10.1   | 7.2    | 9.3    | 6.5    | 7.6             |
| S.....                                 | 1.0                 | 1.6    | 1.4             | 1.0    | 1.2    | 1.1    | 1.2    | 1.0    | 1.7    | 0.9             |
| Free swelling index <sup>1</sup> ..... | 8.0                 | 7.5    | <sup>2</sup> NC | 8.0    | 7.5    | 7.0    | 7.5    | 8.0    | 2.5    | <sup>2</sup> NC |
| Heating value, B.t.u./lb.....          | 14,160              | 13,980 | 13,440          | 13,900 | 13,430 | 13,300 | 13,750 | 13,900 | 13,680 | 13,660          |

<sup>1</sup> American Society of Testing Materials, Standard Test Method for the Determination of the Free Swelling Index of Coal, ASTM Test D-720-57.

<sup>2</sup> NC=Noncaking.

It will be noted that pretreatment of the caking coal in accordance with the process of the invention, as in Tests Nos. 2 and 11 of the examples, resulted in formation of a char that flowed as freely as raw coal. On the other hand, inadequate treatment at the softening temperature, as in Tests Nos. 4, 6, 8 and 10 results in formation of a char that is fused into one solid mass. In Tests Nos. 1, 3, 5, 7 and 9, the elevated temperature treatment was not sufficient to form the desired char.

It is apparent from the above data that successful pretreatment of caking coal to form a nonagglomerated char requires heating at a controlled rate to insure adequate treatment at the softening temperature of the coal prior to heating through the plastic temperature to form char.

What is claimed is:

1. A method of forming a nonagglomerated char from particles of caking coal, said particles having a size of at least about  $\frac{1}{8}$  inch, which comprises heating said coal in a fixed bed to its softening temperature in flowing contact with a gas containing a small but effective concentration of oxygen, said oxygen concentration being in the range of about 0.5 to about 3.0 percent, and thereafter continuing said contacting while controlling the temperature of said coal so as to raise the temperature of said coal through its plastic range in not less than about 1 hour.

2. The method of claim 1 in which the coal is held at its softening temperature for a period of about 1 to 3 hours.

3. The method of claim 1 in which the particle size of the caking coal is from about  $\frac{1}{8}$  to about  $1\frac{1}{2}$  inches.

4. The method of claim 1 in which the oxygen-con-

taining gas is passed through the bed of caking coal at a velocity of from about 0.6 to about 12 feet per second.

5. The method of claim 1 in which the oxygen-containing gas is a mixture of steam and oxygen.

6. The process of claim 1 wherein said step of controlling the temperature of said coal comprises maintaining said coal at its softening temperature for at least about 1 hour and thereafter rapidly heating said coal through its plastic range.

7. The process of claim 1 wherein said step of controlling the temperature of said coal comprises heating said coal through its plastic range at a substantially uniform rate.

8. The process of claim 1 wherein said coal is contacted with said gas at an elevated pressure.

9. The method of claim 8 in which the pressure is about 300 p.s.i.g.

#### References Cited

##### UNITED STATES PATENTS

|           |         |                  |         |
|-----------|---------|------------------|---------|
| 1,767,778 | 6/1930  | Trent            | 201—9   |
| 1,954,351 | 4/1934  | Dornbrook et al. | 201—9   |
| 2,167,099 | 7/1939  | Benezech         | 201—9 X |
| 2,336,151 | 12/1943 | Kruppa           | 201—9   |
| 2,341,861 | 2/1944  | Fuchs            | 201—9   |
| 2,805,189 | 9/1957  | Williams         | 201—9   |
| 3,094,477 | 6/1963  | Kruppa           | 201—9   |

##### FOREIGN PATENTS

770,930 3/1957 Great Britain.

JOSEPH SCOVRONEK, Primary Examiner.